

# UNITED STATES PATENT OFFICE.

ROBERT S. PERRY, OF CAVE SPRING, GEORGIA.

## COMPOSITION FOR COATING SURFACES OF IRON AND STEEL.

1,147,971.

Specification of Letters Patent. Patented July 27, 1915.

No Drawing.

Application filed March 17, 1913. Serial No. 754,815.

*To all whom it may concern:*

Be it known that I, ROBERT SWAIN PERRY, of Cave Spring, in the county of Floyd and State of Georgia, whose present post-office address is Queen and Stokeley streets, Falls of Schuylkill, in the city of Philadelphia, county of Philadelphia, and State of Pennsylvania, have invented certain new and useful Improvements in Compositions for Coating Surfaces of Iron and Steel, of which the following is specification.

My invention relates to a surfacer containing a mineral hydrocarbon base, in conjunction with a chromium salt of the character and in the condition hereinafter set forth, and its purpose is to prevent or minimize rusting of the iron or steel.

To prepare my surfacer, I preferably take refined asphalt, and heat it to a temperature at which it becomes quite fluid, say at about 200° Fahrenheit. I then diffuse throughout the liquefied asphalt, a water-soluble, or partly water-soluble salt of chromium, in a comminuted and substantially dry condition; that is to say, said salt is employed without water (other than its water of crystallization, if it be employed in crystalline form), and without the use of any vehicle containing aqueous moisture, in the initial formation of the compound which constitutes my invention. The salt is introduced without the introduction or employment of any substantial amount of water in the form of aqueous moisture, in order to maintain the full value of a protective coating, which shall be durable and shall be a good excluder of moisture and other agency of metal decay, but the water of crystallization in a chromium salt does not impair the essential function of said salt in the ultimate compound, and hence for the purposes of the present description, the term "substantially dry," is properly applicable to the salt under these conditions. I prefer to use for this purpose, bichromate of soda, but the normal chromate of soda or potash may be employed. Where the bichromate is used, good results may be obtained by adding two and one-half per cent. thereof, but this amount may be varied, and in some instances as high a proportion as twenty per cent. may be found desirable. This salt may be introduced either in a crystalline form, or in a state of subdivision

fine enough for complete and ready diffusion, or it may be desiccated and comminuted.

The ultimate product should, of course, not contain an injurious quantity of any substance which would tend to stimulate corrosion of the iron or steel, such for instance as the metals which are electro-negative to iron, and hence I use the term "substantially free from rust stimulating substances," as fairly descriptive of the proper characteristic.

The compound thus formed may be allowed to cool, for convenience of handling, and may be used alone, by reheating, or in conjunction with any suitable vehicle not containing rust-stimulating substances. Its intended purpose is as a surfacer for iron or steel, whether applied as a coating by means of a brush or other distributing means, or by dipping.

Instead of asphalt any other suitable mineral hydrocarbon base, such as coal tar, paraffin, or any bitumen or pyrobitumen, which is sufficiently viscous to adapt it to be used as a surfacer, and which is substantially free from rust-stimulating ingredients, may be employed in conjunction with the chromic salt. I use the term viscous as an appropriate one to indicate the spreading quality, adhesiveness and tenacity which are characteristic of the above mentioned mineral hydrocarbons when heated, or employed in conjunction with a suitable flux or vehicle.

I believe that the rust-inhibiting qualities of the above described surfacer, are largely due to the fact that the chromium salt, being very completely diffused, in a comminuted condition, throughout the bituminous material, is primarily accessible to any water or aqueous moisture which penetrates the latter, and, being water-soluble, or partly water-soluble, it is taken up by the water or moisture, sufficiently to be carried along with it, to any point of contact with the iron or steel, which may be attained by the water or moisture. Thus the antidote to rust is directly presented at the region where its action is needed, by means of the water or aqueous moisture, which would otherwise tend to produce corrosion. It must be understood, however, that I do not intend to make the above mentioned theory, a part of the essence of my invention, but simply pre-

2  
sent it as a possible explanation of the rust-inhibiting action, which I have found to occur.

Having thus described my invention, I claim:

1. The hereinbefore described surfacer, consisting of a substantially viscous hydrocarbon base in conjunction with a chromic salt, diffused therethrough in a comminuted and substantially dry condition, said compound being substantially free from rust-stimulating substances.
- 10 2. The hereinbefore described surfacer, con-

sisting of a substantially viscous asphalt base in conjunction with a chromic salt, diffused therethrough in a comminuted and substantially dry condition, said compound being substantially free from rust-stimulating substances.

15 In testimony whereof, I have hereunto signed my name at Philadelphia, Pennsylvania, this fifth day of March 1913.

ROBERT S. PERRY.

Witnesses:

JAMES H. BELL,  
E. L. FULLERTON.